

# UNITED STATES PATENT OFFICE.

LOUIS A. CRETSINGER, OF DESHLER, AND JOHN A. WORKMAN, OF CLEVELAND, OHIO.

## TIMBER-PRESERVING COMPOSITION.

1,276,725.

Specification of Letters Patent.

Patented Aug. 27, 1918.

No Drawing.

Application filed November 20, 1916. Serial No. 132,292.

To all whom it may concern:

Be it known that we, LOUIS A. CRETSINGER, and JOHN A. WORKMAN, citizens of the United States, residents, respectively, of

5 Deshler, county of Henry, and State of Ohio, and Cleveland, county of Cuyahoga, and State of Ohio, have invented a new and useful Improvement in Timber-Preserving Compositions, of which the following is a 10 specification, the principle of the invention being herein explained and best mode in which we have contemplated applying that principle, so as to distinguish it from other inventions.

15 Our invention relates to the preservation of timber, its object being to treat timber in an economical and efficient manner with an improved timber preserving composition so as to enable it to resist chemical or other 20 actions to which it may be subjected in the course of its use.

The said invention consists of the means and steps hereinafter fully described and particularly set forth in the claims.

25 In utilizing our above-described invention, we first take the wood to be treated and bore in same a number of holes of a size and distance apart depending upon the size of the timber to be treated. For instance, in 30 the case of railroad ties, we prefer to bore one hole at each end of the tie and two holes in that part of the tie which would lie between the rails and on the top, said holes to be about  $\frac{3}{4}$ " in diameter and about 3" or 4" deep. After these holes have been bored, we inject into same a composition consisting of sixteen (16) parts of sodium chlorid (common salt), six (6) parts of powdered arsenic as popularly known, really arsenic trioxid, and one (1) part of mercuric chlorid (corrosive sublimate). An amount of this

40 mixture is injected into each hole which will fill it to such a point so as to permit a suitable plug to be inserted to stop the hole. 45 Such plug is inserted in each hole, and the material is allowed to remain in place. After a suitable length of time the preserving composition disseminates itself throughout the fibers of the timber and eventually reaches all parts thereof. Although the exact proportions given have been found by us to be the best, they may be somewhat varied

and still satisfactorily accomplish the purpose of our invention, the variation in the mercuric chlorid, which, in addition to ass- 55 sisting in the preservation, also spreads or scatters the composition through the treated wood, being from one-half ( $\frac{1}{2}$ ) of one (1) part to two (2) parts, in the sodium chlorid being from twelve (12) to twenty (20) 60 parts, and in the arsenic trioxid being from four (4) to eight (8) parts.

We have found that timber so treated, particularly railroad ties, pilings, etc., successfully resists all ordinary chemical ac- 65 tions to which the timber may be subjected, becomes hardened, resists tendencies to check and crack and renders efficient service for a greatly increased length of time over that furnished by untreated timber subjected to 70 the same uses.

Having fully described our invention, what we claim and desire to secure by Letters Patent is:-

1. A composition of matter for the preser- 75 vation of timber, consisting of an admixture of a major portion of sodium chlorid, with an arsenical compound, and a mercuric compound in sufficient quantity to spread or scatter the composition throughout the tim- 80 ber.

2. A composition of matter for the preser- 85 vation of timber, consisting of an admixture of a major portion of sodium chlorid, with an arsenic oxid, and an amount of mercuric chlorid sufficient to spread or scatter the composition throughout the timber.

3. A composition of matter for the preser- 90 vation of timber, consisting of an admixture of from twelve to twenty parts of sodium chlorid, four to eight parts of arsenic trioxid and one half part to two parts of mercuric chlorid.

4. A composition of matter for the preser- 95 vation of timber, consisting of an admixture of substantially sixteen parts of sodium chlorid, six parts of arsenic trioxid and one part of mercuric chlorid.

5. A method of preserving wood which consists in boring holes in the wood at suit- 100 able distances from each other, inserting a preserving composition in said holes consisting of a major portion of sodium chlorid, with an arsenical compound, and a mercuric

②  
compound in sufficient quantity to spread or scatter the composition throughout the wood, and then plugging the holes and permitting the wood so treated to retain the preserving composition so placed until it becomes impregnated therewith.

Signed by me, this 16th day of November, 1916.

LOUIS A. CRETSINGER.

Signed by me this 16th day of November, 1916.

JOHN A. WORKMAN.